

# UNITED STATES PATENT OFFICE.

JOHN H. HALL, OF NEW YORK, N. Y., ASSIGNOR TO TAYLOR WHARTON IRON & STEEL COMPANY, OF HIGH BRIDGE, NEW JERSEY, A CORPORATION OF NEW JERSEY.

## PROCESS OF PRODUCING STEEL IN SIDE-BLOWN CONVERTERS.

1,249,075.

Specification of Letters Patent.

Patented Dec. 4, 1917.

No Drawing.

Application filed March 17, 1914. Serial No. 825,404.

To all whom it may concern:

Be it known that I, JOHN H. HALL, a citizen of the United States, and resident of New York, in the county of New York and 5 State of New York, have invented certain new and useful Improvements in Processes of Producing Steel in Side-Blown Converters, of which the following is a specification.

10 This invention relates to a pneumatic process of producing steel from cast iron together with steel scrap or other available forms of ferruginous material, and has in view the oxidation of the carbon, silicon and manganese by lateral air blowing, the main 15 feature being the regulation of the slag formed at successive stages of the operation, so that substantially no overflow or boiling over shall take place, as will now be explained, reference being had to the following specification and claims.

For many purposes it is highly advantageous to use a side blown converter rather than a bottom blown one, owing to the lower 25 cost of the former and its accessories, and for other purposes it is almost essential because in a side blown converter the metal may be brought up to a higher temperature than in a bottom blown one or in an open 30 hearth furnace. However, the use of a side blown converter often is connected with certain difficulties not met with in the use of a bottom blown converter and which 35 difficulties it is the purpose of this invention to overcome.

In a bottom blown converter the material is vigorously agitated, so that the action 40 proceeds uniformly, whereas in a side blown converter the agitation is much less active, from which fact great irregularity in operation often results, causing metal and slag to overflow or boil over from time to time, whereby loss of time and material and great 45 inconvenience is occasioned. For this reason the use of the side blown converter has been much restricted, especially in the treatment of certain residues in which the manganese is relatively high in proportion to the silicon.

50 My process overcomes these difficulties, thus making side blown converters available where hitherto their use was impossible. I accomplish this result by a certain regulation in the quantity of the slag and

percentage of its constituents formed during the operation. 55

Thus, although at times iron is blown in these vessels which contains as much as .5% of manganese or even more, yet as a general rule it has been found that metal 60 of which the silicon content is from about 1 to 2.5% cannot be blown without difficulties if it contains more than about .8 to 1% of manganese. The reason for this is that when the manganese content of such 65 a mixture is above the figure given, the overflow or boiling over of slag and frequently of metal from the converter is greater than is the case when metal low in manganese is blown; and occasions not only 70 serious inconvenience in the handling of the vessel, but frequently a serious loss of metal.

The cause of the boiling over in a side blown vessel appears to be as follows: When the silicon content of the mixture is such 75 in proportion to the manganese content that the  $\text{SiO}_2$  resulting from the oxidation of the silicon by the blast of air, is considerably in excess of the molecular proportion of the  $\text{MnO}$  resulting from the oxidation of 80 the manganese by the blast of air, the slag, which is composed essentially of  $\text{SiO}_2$  and  $\text{MnO}$ , (plus a greater or less amount of  $\text{FeO}$  resulting from the oxidation of some 85 of the iron of the metal), has so high a melting point that it is not freely fluid during the greater part of the blow.

In the oxidation of the bath, the silicon and manganese of the surface layer are first oxidized, (approximately at the same time), 90 and form a slag composed largely of  $\text{SiO}_2$  and  $\text{MnO}$ . If the  $\text{SiO}_2$  so far exceeds the  $\text{MnO}$  that the slag is not freely fluid at the temperature existing at that time in the vessel, the slag combines with a greater or 95 less amount of  $\text{FeO}$ ; the oxidation of iron to  $\text{FeO}$  occurring more rapidly as the silicon and manganese of the bath are reduced; also as the temperature rises; and as the capacity of the slag for retaining  $\text{FeO}$  is 100 greater or less,—i. e. the greater the excess of  $\text{SiO}_2$  over  $\text{MnO}$ , the greater the capacity of the slag for  $\text{FeO}$ , and vice versa.

Thus in blowing metal containing say 2% of silicon and .5% of manganese, the 105 combination of  $\text{FeO}$  with the slag continues until the slag becomes freely fluid; and as the carbon of the surface layers of the bath

is oxidized to CO, both before the iron begins to oxidize in considerable quantities and also during the oxidation of the iron, more iron is oxidized and enters the slag than could be the case if the slag were in constant contact with a metal containing a high proportion of carbon. The slag, therefore, becomes saturated with FeO, so that it is for the time being quite fluid and highly oxidizing.

As the bath of metal and slag is agitated to a considerable extent by the blast impinging upon its surface at a slight angle, there is a tendency to mix the slag with the metal. When the slag is highly fluid this tendency is increased. Moreover, at the time when a great proportion of the silicon, manganese and carbon have been oxidized from the surface layers of the metal so that iron begins to be oxidized quite strongly, the carbon of the underlying portions of the bath will continue to be carried upward by gravity, diffusion and convection, and there will consequently be an increase in the content of carbon in the surface layer of the metal. When the carbon content of the surface layer is increased in this way to a sufficiently high point, and when the slag, (which becomes very fluid at about the same time), is mixed with the surface metal by the action of the blast, a point is presently reached where a strong reaction begins to take place between the FeO of the slag and the carbon of the metal, according to the formula:  $FeO + C = Fe + CO$  (or some similar formula). This reaction is often so violent that it assists greatly in causing a large portion of the bath to be violently agitated, and hence in a few moments after the reaction starts, a great deal of the metal is intimately mixed with the slag, and reacts with it, so that a great volume of CO is generated and causes both metal and slag to froth up and fill the upper portions of the vessel, and frequently to boil over, in greater or less amount. In these boilings, a loss frequently occurs not only of slag but also of metal.

This reaction, once started, continues until the FeO of the slag is reduced to such an extent that the slag loses its oxidizing power very largely, and is no longer freely fluid. A certain amount of the FeO will remain in the slag because the affinity between the  $SiO_2$  of the slag and that percentage of FeO is too strong to be overcome by the affinity of carbon for the O of the FeO. When this point is reached the reaction ceases, the boiling subsides, and the bath, whose composition has been rendered more or less uniform by the agitation produced by the boil, continues to be subjected to the oxidizing action of the blast, which is always confined largely to that portion of the bath constituting the surface layer. The oxygen of

the blast again oxidizes silicon, manganese, carbon and iron, from the upper layer of the bath, and the same sequence of events tends to occur a second and sometimes a third, fourth or fifth time.

It is known that such a slag as is produced in the Bessemer process is governed by certain laws based on the constitution of the material treated; and in particular that the ratio of the weight of the  $SiO_2$  to the sum of the weights of the  $MnO$  and the  $FeO$  tends to assume a certain value, varying with the temperature and other conditions, a value corresponding to a slag of minimum melting point. It appears, moreover, that the relative amounts of  $FeO$  and  $MnO$  present in the slag do not affect this ratio between the weight of  $SiO_2$  and the sum of the weights of  $FeO$  and  $MnO$ , which governs the composition of the slag of minimum melting point. This tendency of the slag to absorb  $FeO$  and  $MnO$  up to a certain sum, is offset to a greater or less extent by the tendency of the  $FeO$  of the slag to react with the carbon of the bath, as has been described. Hence, we see that if a bath is treated containing the usual high proportion of silicon, say 2%, and in addition manganese to the extent of some 1% (Example 1), a slag will be produced consisting of  $SiO_2$ ,  $MnO$  and  $FeO$ , which will become fluid upon the absorption of an amount of  $FeO$  less than the amount necessary to render fluid the slag resulting from the oxidation of the silicon and manganese of a bath containing much silicon and very little manganese, as for instance, 2% silicon and .50% manganese (Example 2). It is evident, therefore, that in blowing the first mixture, the period during which the oxidation of Fe from the metal and its absorption as  $FeO$  by the slag takes place, will be shorter than the corresponding period in the second mixture; because after the elimination of the silicon and manganese from the surface layer of the metal by oxidation has taken place, an amount of  $FeO$  will be absorbed sufficient to make the slag freely fluid and oxidizing; and this amount of  $FeO$  will be less in Example 1, than in Example 2. The reaction between the  $FeO$  of the slag and the carbon of the bath, will occur sooner in Example 1, in which the manganese is about 1% and the silicon about 2% than in Example 2, in which the manganese is about .5% and the silicon about 2%, because the silicon and manganese are oxidized from the metal approximately at the same time, and hence the total time elapsing between the beginning of the blow and the time when the slag becomes freely fluid and oxidizing will be less in Example 1 than in Example 2; because less Fe need be oxidized to make the slag fluid, in Example 1 than in Example 2. The boiling, therefore, will take place

70

75

80

85

90

95

100

105

110

115

120

125

130

earlier in Example 1 than in Example 2; and by the same reasoning, the period between the first and the second boils, and between the second and third boils, etc., will 5 be similarly shorter in Example 1 than in Example 2. Hence, in blowing a bath such as indicated in Example 1, the boils will occur more frequently; and it has been found by experience that they will be violent and 10 will result in a considerable loss of metal.

As before stated, the object of the present invention is to enable the steel maker to blow in a side-blown converter, a bath of metal consisting of molten pig iron with 15 manganese steel scrap with or without mixtures of ordinary steel scrap, or special varieties of pig iron or steel high in manganese, which shall contain in combination with silicon, manganese in proportion equal 20 to or greater than those that have been found in the past to cause the explosive overflow which I have described. I have found by experiment that if the proportions of silicon and manganese in the fluid bath 25 of metal are such that a slag is produced by their oxidation to  $\text{SiO}_2$  and  $\text{MnO}$  which is freely fluid practically from the time when it begins to be formed, and such that the necessary amount of heat is produced by their 30 oxidation, the metal can be blown in a side blown converter of any of the usual types without the serious explosive overflow or boiling over which hitherto has accompanied the blowing in a side blown converter of 35 metal containing a considerable proportion of manganese, in all previous experiments.

In order to blow such a bath successfully, the manganese and silicon must be in such proportion that the  $\text{SiO}_2$  and  $\text{MnO}$  produced by their oxidation are in the proportion approximately of  $\text{SiO}_2$ —40%, and  $\text{MnO}$ —60%, which corresponds practically to 4 molecules of  $\text{SiO}_2$  to 5 molecules of  $\text{MnO}$ ; and the amounts of silicon and manganese must be such as to produce sufficient heat to maintain both metal and slag at the requisite temperature.

It must be understood that the exact proportion of  $\text{SiO}_2$  and  $\text{MnO}$  in the slag will 50 vary according to the temperature existing in the vessel at the time, and with other factors; so that it may be found that a proportion of  $\text{MnO}$  much lower, or much higher, than 60% may be essential in order that the 55 slag may be fluid. I do not confine myself to exact proportions of  $\text{SiO}_2$  and  $\text{MnO}$ , but vary this proportion to suit the particular case in such a way that the slag produced in the blowing shall be freely fluid during the 60 greater part of the operation.

I do not confine myself, moreover, to any particular proportion of silicon in the bath; the total amount of silicon may be such as is ordinarily found in the metal treated in a 65 side-blown vessel. It may be as low as .90%

or even lower, and it may be as high as 2.5% or even higher. But for any particular proportion of silicon in the bath, the proportion of manganese in the bath must be such that the slag resulting from the 70 oxidation of the silicon and manganese shall be freely fluid practically from the time it begins to be formed; and that the heat produced by the oxidation of the silicon and manganese shall be sufficient to maintain the 75 metal and slag at the necessary temperature.

The proportion of the  $\text{SiO}_2$  and  $\text{MnO}$  in the slag resulting from the oxidation of the silicon and manganese of the metal must be 80 such as to result in a freely fluid slag; I have found that the proportions 40%  $\text{SiO}_2$  and 60%  $\text{MnO}$  are suitable in certain cases; but as already stated, I do not confine myself to that exact proportion, and the  $\text{MnO}$  may 85 be so high that at any given temperature there is more of it present than that necessary to produce a fluid slag; and if the conditions are such that a slag with less than 60%  $\text{MnO}$  will be fluid, I may use a much 90 lower proportion of  $\text{MnO}$  in the slag.

In blowing such a mixture, it is evident that after the silicon, manganese and carbon in the surface layer of the metal are so far eliminated that the oxidation of iron in 95 those layers begins to take place in considerable amount, the slag, which is already fluid, and in which there is already enough  $\text{MnO}$  to satisfy the  $\text{SiO}_2$  without the addition of much  $\text{FeO}$ , will react with the bath 100 as soon as even a very small amount of  $\text{FeO}$  has been absorbed. This will be true because the slag being freely fluid, tends to mix with the metal throughout the operation; and though in some cases iron will be 105 oxidized and enter the slag as  $\text{FeO}$  in appreciable amounts, before the carbon of the surface layer has become high enough by the mixing of the bath to react with the  $\text{FeO}$  of the slag; yet it has been found that 110 the reaction takes place so early in the operation and at a time when the slag contains so little  $\text{FeO}$ , that the reaction does not result in the overflow of slag and metal from the converter.

A further useful feature of this process is that advantage is taken of the heat of combination of the manganese of the metal, in addition to the heat of the combination of the silicon of the metal, and this is utilized, 120 in raising the temperature of the bath, and of course also of the slag.

The fluid slags, high in  $\text{MnO}$ , produced by blowing such mixtures as are the subject of this specification, are more severe upon 125 the lining of the converter than the less fluid slags produced in regular practice. The reason for this is that in the majority of cases the lining of the vessel is composed of silica rock, mica schist, ganister or other 130

4

material of like nature, in which  $\text{SiO}_2$  largely predominates. When this lining is brought in contact with a fluid slag containing a high proportion of  $\text{FeO}$ ,  $\text{MnO}$ , or both, if the proportion of these bases in the slag is greater than that necessary for maximum fluidity, a considerable amount of  $\text{SiO}_2$  will be absorbed by the slag from the lining material, with resultant wear of the lining. 5

10 In the process of blowing, it is at different times the case that the slag at one or more points of contact with the lining will be so high in  $\text{MnO}$  or  $\text{FeO}$ , or both, as to corrode the lining in this manner. In the bottom 15 blown type of vessel, this wear upon the lining is naturally greatest at the surface of the bath, where the slag comes in contact with the lining. The twyers being at the bottom of the bath, are less affected than 20 the solid lining of the sides of the vessel, which may be patched comparatively easily. In the side blown vessel, however, the twyers are placed in the sides of the vessel, and their mouths are more or less immersed in 25 the slag throughout the operation. Thus it happens that the portion of the lining containing the twyers is corroded to a considerable extent; and thus the twyers and the lining at that point are sometimes cut away 30 more rapidly than is the case in ordinary practice. Because the twyers must not be allowed to become shorter than a certain definite length, it may in some cases be necessary to repair the lining, especially at 35 the twyers, more often in blowing these high manganese mixtures than is the case in ordinary practice. The advantages secured by the process, however, very much more than off-set this trifling disadvantage 40 in the majority of cases.

In proportioning the ingredients of the charge, I may secure the desired amounts of manganese and silicon by the use of a pig iron containing such proportions of the 45 elements in question that it shall, when melted, have the proper relative amounts of silicon and manganese; or I may mix several pig irons containing varying proportions of silicon and manganese, in such relations as to obtain the composition desired; or I may mix one or more such 50 pig irons with appropriate amounts of iron or steel scrap in order to obtain the composition desired; or I may use in combination with such a mixture of one or more pig irons, or of one or more pig irons and one or more kinds of scrap, special varieties of pig iron containing high proportions of manganese, silicon, or both. I may also 55 obtain part of the silicon and manganese in the mixture by the addition to the charge of suitable amounts of ferro-manganese, spiegeleisen, ferro-silicon, silico-spiegel, or other similar alloy. Again, I may obtain 60

a considerable proportion of the manganese 65 of the charge by utilizing steel scrap containing a high proportion of manganese. The exact proportions of these varying ingredients of the charge, and of the silicon and manganese in those ingredients, is immaterial, since it is generally a matter of simple arithmetic to so proportion ingredients of varying composition that the sum total of the manganese and the silicon of the mixture shall be what is desired. 70

75 Thus, for instance, if it is desired to treat in the converter 4,500 pounds of metal containing 1.90% of silicon, and 4.18% of manganese; and if this metal is to be melted in the cupola, so that a loss of silicon and 80 manganese must be allowed for in melting the ingredients of the charge; I may find it desirable to so proportion those ingredients that they shall contain an average of 2.03% of silicon and 5.34% of manganese. 85 By charging to the cupola 2,100 pounds of steel scrap containing .3% of silicon and 12% of manganese; 2,100 pounds of pig iron containing 3.97% of silicon and .32% of manganese; 445 pounds of pig iron containing 2.07% of silicon and .3% of manganese; and 255 pounds of steel scrap containing .30% of silicon and .75% of manganese, I shall secure in the mixture the 90 average percentage of those elements desired. Of course the weight of metal charged to the cupola must be sufficiently greater than the 4,500 pounds of fluid metal desired, to allow for this loss of silicon and manganese, and also for the loss of a certain amount of iron. As the losses in melting in a cupola are not the same in all cases, 95 it will not be possible to use the exact figures here given in every case; but the behavior of the cupola must be ascertained by experiment, as in any other process. As already stated, the proportions of silicon and manganese in this example are given as examples of compositions which will secure 100 the desired results under the proper conditions. 105

Variations in the proportions and in the total quantity of manganese and silicon may be made, provided that the total quantity is such as to generate sufficient heat of combination to maintain the slag formed in a freely fluid state. 115

The metal or mixture of metals to be treated may be taken from a blast furnace or blast furnaces directly, or may be melted 120 in a cupola, in the vessel in which the air blowing takes place, or in any other known and suitable device.

What I claim as new is:

1. In the pneumatic process of making 125 steel, the improvement which consists in subjecting to lateral air blowing, ferruginous material in which silicon and manganese are

so proportioned that the slag produced by their oxidation shall approximate 60 parts of MnO to every 40 parts of SiO<sub>2</sub> and be workably fluid throughout the blow.

5 2. In the pneumatic process of making steel, the improvement which consists in subjecting to lateral air blowing a ferruginous mixture in which the silicon and manganese are present in such quantity and 10 are so proportioned that by their oxidation there is produced a workably fluid slag containing approximately 60 parts of MnO to every 40 parts of SiO<sub>2</sub>.

15 3. In the pneumatic process of making steel, the improvement which consists in subjecting to lateral air blowing, ferruginous material in which the silicon and manganese are present in such quantity and are so proportioned that the slag produced by their 20 oxidation shall contain approximately 60 parts of MnO to every 40 parts of SiO<sub>2</sub> and that the power of the slag produced to retain FeO in combination is so limited that the FeO practically as fast as formed reacts 25 with the carbon of the metal, whereby the boiling of the bath is practically continuous and the tendency of the bath to boil over is substantially eliminated.

30 4. In the pneumatic process of making steel, the improvement which consists in subjecting to lateral air blowing, a mixture containing steel high in manganese, and pig iron, in which mixture the proportion of 35 silicon to manganese is such that by their oxidation a slag is produced that contains approximately 60 parts of MnO to every 40

parts of SiO<sub>2</sub> and that is workably fluid practically throughout the blow.

5. In the pneumatic process of making steel, the improvement which consists in 40 subjecting to lateral air blowing, a mixture containing steel high in manganese, and pig iron, in which the silicon and manganese are present in such quantity, and are so proportioned that by their oxidation there is 45 produced a workably fluid slag containing approximately 60 parts of MnO to every 40 parts of SiO<sub>2</sub>.

6. In the pneumatic process of making steel, the improvement which consists in 50 subjecting to lateral air blowing, a mixture containing steel high in manganese, and pig iron, in which the silicon and manganese are present in such quantity and are so proportioned that the slag produced by their 55 oxidation shall contain approximately 60 parts of MnO to every 40 parts of SiO<sub>2</sub>, and that the power of the slag produced to retain FeO in combination is so limited that the FeO practically as fast as formed reacts 60 with the carbon of the metal, whereby the boiling of the bath is practically continuous and the tendency of the bath to boil over is substantially eliminated.

Signed at New York, in the county of 65 New York and State of New York, this 16th day of March, A. D. 1914.

JOHN H. HALL.

Witnesses:

C. A. O. ROSELL,  
HOWARD E. BROWN.